

[54] **PROCESS FOR CREESEPROOFING CELLULOSE-CONTAINING FABRIC WITH GLYOXAL-UREA-FORMALDEHYDE REACTION PRODUCT AND A BORON COMPOUND**

[75] Inventors: **Ronald Louis Readshaw, South Charleston; George Henry Lourigan, Charleston, both of W. Va.**

[73] Assignee: **Union Carbide Corporation, New York, N.Y.**

[22] Filed: **Mar. 4, 1970**

[21] Appl. No.: **16,565**

[52] U.S. Cl..... **8/115.7, 8/116.3, 8/133, 117/139.4, 260/29.4, 260/70**

[51] Int. Cl..... **D06m 13/40, D06m 15/58**

[58] Field of Search..... **8/116.3, 133, 115.7; 260/29.4; 117/139.4**

[56] **References Cited**

UNITED STATES PATENTS

|           |        |                   |           |
|-----------|--------|-------------------|-----------|
| 3,178,250 | 4/1965 | Ellis et al.....  | 8/120 X   |
| 3,576,591 | 4/1971 | Cusano et al..... | 8/116.3   |
| 3,186,954 | 6/1965 | Hushebeck .....   | 8/116.3 X |
| 2,876,062 | 3/1959 | Torke et al.....  | 8/116.3 X |

FOREIGN PATENTS OR APPLICATIONS

498,763 1/1939 Great Britain ..... 8/116.4

OTHER PUBLICATIONS

"Crease Resisting Fabrics," J. T. Marsh, 1962, pages 74 and 75, Reinhold Publishing Corp. NYC, N. Y.

"An Introduction to Textile Finishing," J. T. Marsh, page 317, 1948, Chapman and Hall, Ltd., London, England.

"Merck Index," 7th, Edition, 1960, page 460, Merck & Co., Rahway, N. J.

Primary Examiner—George F. Lesmes

Assistant Examiner—Harold Wolman

Attorney—James C. Arvantes, Francis M. Fazio and Aldo J. Cozzi

[57] **ABSTRACT**

In combination glyoxal and a boron containing compound selected from the group consisting of the alkali metal borates and boric acid, the combination being incorporable into a resin forming reaction mixture to produce a durable press finish, and an improved process for treating textile fabrics with the same thereby yielding a treated fabric of significantly less discoloration than heretofore known and one exhibiting at the same time, improved strength properties.

**5 Claims, No Drawings**

**PROCESS FOR CREASEPROOFING  
CELLULOSE-CONTAINING FABRIC WITH  
GLYOXAL-UREA-FORMALDEHYDE REACTION  
PRODUCT AND A BORON COMPOUND**

**BACKGROUND OF THE INVENTION**

**1. Field of the Invention**

This invention relates generally to textile fabrics possessing durable press properties and, more particularly, to cellulose and cellulose-containing textile fabrics treated with novel glyoxal durable press finishes in combination with a boron containing compound, whereby the treated textile fabrics exhibit substantially reduced discoloration and improved strength properties.

**2. Description of the Prior Art**

Crease-resistant finishing agents, i.e., durable press finishes for fibrous material, particularly cellulose and cellulose-containing textile fabrics, have recently become widely used, and a large proportion of such materials now provided to the trade have been treated with such finishes for the production of fabrics having durable press characteristics. Cellulose reactants have been among such agents and one currently used durable press finish comprises the reaction product of glyoxal, urea and formaldehyde in an aqueous medium. While this prior art finish, when applied to a cellulose substrate, does impart certain durable press characteristics, to the treated substrate, e.g., dry wrinkle recovery and durable press qualities, the latter properties have been sometimes offset by the discoloration of the treated product and by the loss of fabric strength.

In the past, an attempt has been made to employ boron-containing compounds to overcome the discoloration problem (yellowing) of cellulose attendant upon the alkaline degradation of cellulose in the alkaline treatment thereof with sulfone-type cross linking agents. Moreover, while borate compounds have been known to be used as cross linking catalysts for celluloses, in amounts ranging between about 2 to 4 percent, no color improvement has been achieved therewith. Thus, it would be entirely unexpected that a boron-containing compound, when used in an acidic media or with acidic catalysts in conjunction with glyoxal based cross linking agents (finishes) applied to cellulosic fabrics, would overcome the prior art problems of discolored and weakened fabrics.

**SUMMARY OF THE INVENTION**

In accord with the invention, it has been discovered that a combination of glyoxal-based durable press finishes, formed by reacting glyoxal, urea and formaldehyde in an aqueous medium, and a boron-containing compound selected from the group consisting of alkali metal borates and boric acid in aqueous medium when applied to a suitable cellulose or cellulose containing textile fabric produces a fabric of significantly less discoloration and of improved strength.

The boron-containing additive may be incorporated into the glyoxal solution per se, in amounts between about 0.5 and about 20 weight percent, preferably between about 6 and about 14 weight percent, and still more preferably, about 9 weight percent; or, it may be added to an aqueous mixture of glyoxal, urea and formaldehyde or, alternatively, the additive may be placed into a suitable pad bath solution for application to the desired fabric. It has been found that the boron additive

in the pad bath solution should be in amounts ranging between about 0.01 and about 1.5 weight percent. Maximum reduction of discoloration of the finished treated fabric has been found to be at the level of about 0.5 weight percent boron additive in the pad bath solution. Indeed, amounts below 0.01 percent boron additive and above 1.5 percent boron additive show sharply increased discoloration levels. Thus, the concentration of boron additives is critical.

In terms of fabric content, the boron compound is normally present in amounts ranging between about 0.05 and 1.5 weight percent, based on the weight of fabric, preferably between about 0.125 and about 1.0 weight percent, and still more preferably between about 0.25 and about 0.5 weight percent, using a wet pick-up of 50 to 100 percent.

**DESCRIPTION OF THE SPECIFIC EMBODIMENTS**

In the usual practice of the invention, a durable press resin forming solution is prepared by reacting glyoxal, urea and formaldehyde in any desired sequence, and employing the resultant reaction product 1,3-dimethylol-4,5-dihydroxy-2-imidazolidone in an aqueous medium. This is a typical commercial resin forming solution presently utilized for durable press finished products.

As earlier indicated, an additive comprising a boron-containing compound selected from the group consisting of alkali metal borates and boric acid may be added either to the glyoxal solution per se or to the glyoxal, urea, formaldehyde reaction mixture in aqueous solution. Illustrative of the boron-containing compounds are the following: boric acid, sodium tetraborate, sodium metaborate, sodium perborate, potassium tetraborate and potassium pentaborate, merely to name a few. Particularly preferred additives on the basis of over-all performance have been found to be sodium tetraborate and sodium metaborate.

Alternatively, the boron additive is incorporated into a standard pad bath solution containing the finish, i.e., the glyoxal-based resin forming solution just described; a catalyst, such as zinc nitrate or magnesium chloride; a surfactant, such as Tergitol 15-S-9; a softener, such as Mykon SF; a hand builder such as polyvinyl acetate; and water. The fabric to be treated is passed through the solution for the purpose of wet pickup of the pad solution ingredients and then placed on pin tenter frames. Thereafter, the fabric is usually dried at an elevated temperature to remove the water therefrom. While drying can be accomplished by simply allowing the fabric to remain in contact with air at room temperature, it is preferred to dry the fabric at a temperature of from about 250° to 300°F. for a period of about 30 to about 120 seconds, the higher temperatures generally being employed in conjunction with the shorter drying times.

After this drying step, the fabric is cured by heating at a temperature sufficient to promote the reaction of resin forming solution with the fabric so as to bind it chemically thereto and thereby impart the durable press properties. The curing can be carried out at temperatures from about 300° to 360°F. for periods ranging from about 30 seconds to 15 minutes, with the higher temperatures generally being employed in conjunction with the shorter heating times. Subjecting the treated textile fabric to a two-step curing procedure involving a pre-curing period and a post-curing period, as herein-

before described, is preferred, but it is not a critical feature of the process of this invention. It will be obvious to one skilled in the art that both drying and curing could be accomplished in a single operation or sequential operation.

The term "cellulose and cellulose-containing textile fabrics" as used throughout the specification and claims is intended to include fabrics, whether woven, non-woven or knitted, and garments or other articles made from such fabrics. Fabrics containing cellulose, 10 regenerated cellulose, and mixtures of the two are intended to be within the scope of the present invention. Illustrative of the textile fabrics to which this invention relates are cotton fabrics, linen fabrics, rayon fabrics, fabrics consisting of blends of cotton, linen or rayon fibers, and fabrics consisting of blends of cellulosic fibers and non-cellulosic fibers, such as, for example, polyester or polyamide fibers.

Thus, by subjecting any one of the above listed fabrics to a textile treating solution containing the glyoxal based resin forming mixture and the boron containing compound, it has been found that textile fabrics are obtainable, which exhibit substantial reduction in discoloration of the treated fabric, a stronger fabric and, as an incidental feature, reduction in shade change. As indicated, the amount of boron-containing additive is in the range between about 0.01 and about 1.5 weight percent of the pad bath treating solution. Maximum reduction of discoloration of the finished treated product has been found to be at the level of about 0.5 weight percent additive.

Evaluation of the textile fabrics subjected to the process of this invention was made in accordance with accepted test procedures of the ASTM (American Society For Testing Materials), or the AATCC (American Association of Textile Chemists and Colorists), or by procedures that are fully described herein. The following tests were conducted:

|                                    |                                                                       |
|------------------------------------|-----------------------------------------------------------------------|
| Dry Wrinkle Recovery               | - AATCC Tentative Test Method 66-1959T                                |
| Tensile Strength                   | - ASTM Method D-1682 (Grab)                                           |
| Tear Strength                      | - ASTM Method D-1424-59 (Elmendorf)                                   |
| Damage Caused by Retained Chlorine | - AATCC Tentative Test Method 114-1967                                |
| Durable Press Rating               | - AATCC Test Method- 124                                              |
| Yellowness Index                   | - Measured with a Hunterlab Model D-40 reflectometer excluding filter |
|                                    | Yellowness = $\frac{\text{Green-Blue Reflectance}}{100}$              |
|                                    | Increasingly positive numbers indicate increasingly yellow fabric     |

The following definitions will also be applicable in the Examples and wherever appearing in the specification:

|                 |                                                                                                            |
|-----------------|------------------------------------------------------------------------------------------------------------|
| Catalyst X-4    | - An acetic acid solution of zinc nitrate hexahydrate.                                                     |
| Mykon SF        | - A nonionic paraffin-free polyethylene emulsion softening agent.                                          |
| Tergitol 15-S-9 | - A C <sub>11</sub> to C <sub>15</sub> linear chain alcohol-ethylene oxide adduct used as a wetting agent. |

Boron salts used to effect improvements in the fabric performance properties can be introduced into the treating bath by a number of different procedures, as have already been indicated. One method involves the addition of the boron additive directly to the pad bath solution along with the other pad bath components. No adverse effects have been observed when the boron salts have been added to the durable press finish. Alternatively, another method involves the addition of the boron-containing material to a durable

press finish and marketing the finish containing the additive, whence it will be eventually added to the pad bath solution. In yet another alternative method of introducing the boron salt to a durable press treating bath, the boron salt is added to a raw material, e.g., glyoxal, that is used to make a durable press finish. In other words, sodium metaborate can be added to glyoxal, the glyoxal used to make a durable press finish and the finish used to treat the fabric to impart durable press properties thereto. The various alternative methods of introducing the boron containing additive will be better understood in conjunction with the following specific examples. 1-7.

#### Example 1

The pH of a mixture of 170 grams of 40 percent glyoxal (1.17 moles) and 187.6 grams of 37.5 percent uninhibited formaldehyde (2.34 moles) was adjusted to 5.5 with 7.4 grams of a 30 percent aqueous sodium acetate solution; 70.4 grams of urea (1.17 moles) was then added and the pH of the mixture raised to 7.0 with 1.3 grams of a 10 percent aqueous sodium hydroxide solution and maintained at this pH for the remainder of the reaction with the periodic addition of 14.8 grams of the 10 percent aqueous sodium hydroxide solution. The temperature of the reaction mixture was raised to 60°C. and maintained at this temperature for 1½ hours. The reaction product, 1,3-dimethylol-4,5-dihydroxy-2-imidazolidone, was cooled to room temperature and 24.0 grams of distilled water was added to make a 45 percent solution. The formaldehyde content of the 45 percent product was 0.59 percent, and pH 7.0 and the color 100 (Pt), ASTM D1209-62.

#### Example 2

The pH of a mixture of 170 grams of 40 percent glyoxal (1.17 moles) and 187.6 grams of 37.5 percent uninhibited form-aldehyde (2.34 moles) was adjusted to 5.5 with 7.6 grams of a 30 percent aqueous sodium acetate solution; 70.4 grams of urea (1.17 moles) was then added and the pH of the mixture raised to 7.0 with 1.3 grams of a 10 percent aqueous sodium hydroxide solution. Six and one-half grams of sodium tetraborate was added intermittently with 13.3 grams of 24 percent sodium hydroxide. The intermittent addition of base is necessary to maintain the pH of the reaction mixture between 6.0 and 7.0. After the sodium tetraborate had been added, the temperature of the reaction was raised to 60°C. and the pH maintained at 7.0 for 2 hours, after which another 6.5 grams of sodium tetraborate was added. The pH of the reaction was maintained at 7.0 during and after the reaction period by the addition of 31.8 grams of 10 percent sodium hydroxide. The formaldehyde content of the reaction product was nil, the color 65 (Pt) and the pH 7.0.

#### Example 3

The procedure used to make the finish of this example was the same as that used to make the finish of Example 2 with the exception of boric acid being used instead of sodium tetraborate. The formaldehyde content of the present finish was nil, the color 60 (Pt) and the pH 7.0.

#### Example 4

The pH of a mixture of 170 grams of 40 percent

glyoxal (1.17 moles) and 187.6 grams of 37.5 percent uninhibited formaldehyde (2.34 moles) was adjusted to 5.5 with 7.3 grams of a 30 percent aqueous sodium acetate solution; 70.4 grams of urea (1.17 moles) was then added and the pH of the mixture raised to 7.0 with 1.3 grams of a 10 percent aqueous sodium hydroxide solution and maintained at this pH for the remainder of the reaction with the periodic addition of 14.8 grams of the 10 percent aqueous sodium hydroxide solution. The temperature of the reaction mixture was raised to 60°C. and maintained at this temperature for 2 hours. The reaction product, 1,3-dimethylol-4,5-dihydroxy-2-imidazolidone, was cooled to room temperature and enough distilled water was added to make a 45 percent solution. The formaldehyde content of the 45 percent product was 0.30 percent, the pH 7.0 and the color 65 (Pt).

### Example 5

To 170 grams of 40 percent glyoxal (Union Carbide Corporation) was added 15 grams of sodium metaborate. The mixture remained at ambient temperature (24°C.) for 3 days and was then used in the following manner to make a glyoxal-based finish. The pH of a mixture of 170 grams of 40 percent glyoxal (1.17 moles), to which had been added 15 grams of sodium metaborate and 187.6 grams of 37.5 percent uninhibited formaldehyde (2.34 moles) was adjusted to 5.5 with 5.3 grams of a 30 percent aqueous sodium acetate solution; 70.4 grams of urea (1.17 moles) was then added and the pH of the mixture raised to 7.0 with 1.0 gram of a 10 percent aqueous sodium hydroxide solution and maintained at this pH for the remainder of the reaction with the periodic addition of 12.2 grams of the 10 percent aqueous sodium hydroxide solution. The temperature of the reaction mixture was raised to 60° C. and maintained at this temperature for 1½ hours. The reaction product, 1,3-dimethyl-4,5-dihydroxy-2-imidazolidone, was cooled to room temperature and enough distilled water was added to make a 45 percent solution. The formaldehyde content of the 45 percent product was 0.20 percent, the pH 7.0 and the color 45 (Pt).

In order to illustrate that this invention is applicable to other commercially available glyoxal material, the finishes of Examples 6 and 7 were prepared using Nobel Bozel glyoxal, another commercially available glyoxal.

### Example 6

### **The pH of a mixture of 170 grams of Nobel Bozel 40**

percent glyoxal (1.17 moles) and 187.6 grams of 37.5 percent uninhibited formaldehyde (2.34 moles) was adjusted to 5.5 with 6.8 grams of a 30 percent aqueous sodium acetate solution; 70.4 grams of urea (1.17 moles) was then added and the pH of the mixture raised to 7.0 with 1.2 grams of a 10 percent aqueous sodium hydroxide solution and maintained at this pH for the remainder of the reaction with the periodic addition of 14.4 grams of the 10 percent aqueous sodium hydroxide solution. The temperature of the reaction mixture was raised to 60°C. and maintained at this temperature for 2 hours. The reaction product, 1,3-dimethylol-4,5-dihydroxy-2-imidazolidone, was cooled to room temperature and enough distilled water was added to make a 45 percent solution. The formaldehyde content of the 45 percent product was 0.30 percent, the pH 7.0 and the color 90 (Pt).

### Example 7

The procedure used to make the finish of Example 6 was the same used to make the finish of the present example with the exception that 15.0 grams of sodium metaborate had three days previously been added to 170.0 grams of Nobel Bozel glyoxal and this material was used to make the present finish. The formaldehyde content of the finish was 0.2, the color 70 (Pt) and the pH 7.0.

30 Each of the finishes made by the procedures of 1 through 7 were then individually applied to white cotton 136 x 64 broadcloth which had been desized, scoured, bleached and mercerized by padding through a laboratory padder at a wet pick-up of 75 percent. The fabrics were placed on pin tenter frames, dried at 300°F. for 1.5 minutes and cured for 1.5 minutes at 340°F. or 15 minutes at 320°F. in a laboratory oven.

Table 1 constituting Examples 8 to 14 lists the treating or pad bath formulations.

40 Tables II and III detail the fabric performance properties shown by fabrics treated by the bath formulations illustrated by Examples 8 to 14 respectively. In Tables II and III, the series denoted by Examples 8a, 9a, 10a show the effect of adding the sodium tetraborate or 45 boric acid to the reaction of glyoxal, urea and formaldehyde to make the glyoxal-based finish used to impart durable press properties to the fabrics. The series denoted by Examples 11a, 12a, 13a and 14a show that sodium metaborate can be added to glyoxal which is subsequently used to make a glyoxal-based durable press 50 finish and still yields the desired improvements in the fabric performance properties.

TABLE I.—TREATMENT BATH FORMULATION

TABLE II.—FABRIC PERFORMANCE PROPERTIES AT A CURE TIME OF 1.5 MINUTES AT 340° F.

| Property                                                          | Treatment |         |         |         |         |         |         |
|-------------------------------------------------------------------|-----------|---------|---------|---------|---------|---------|---------|
|                                                                   | Ex. 8a    | Ex. 9a  | Ex. 10a | Ex. 11a | Ex. 12a | Ex. 13a | Ex. 14a |
| Yellowness index.....                                             | .067      | .026    | .030    | .036    | .029    | .037    | .032    |
| Tear strength (warp/fill) grams.....                              | 400/208   | 704/464 | 672/448 | 560/352 | 592/400 | 528/352 | 608/416 |
| Tensile strength (fill) pounds.....                               | 19        | 26      | 25      |         |         |         |         |
| Dry wrinkle recovery (warp-fill) degrees.....                     | 300       | 283     | 278     | 298     | 302     | 297     | 274     |
| Durable press rating tumble dry/spin dry.....                     | 3.5/3.1   | 3.4/3.0 | 3.4/3.0 |         |         |         |         |
| Damage caused by retained chlorine, percent loss in strength..... | 2.75      | 4.30    | Nil     |         |         |         |         |

TABLE III.—FABRIC PERFORMANCE PROPERTIES AT A CURE TIME OF 15 MINUTES AT 320° F.

| Property                                                          | Treatment |         |         |         |         |         |         |
|-------------------------------------------------------------------|-----------|---------|---------|---------|---------|---------|---------|
|                                                                   | Ex. 8a    | Ex. 9a  | Ex. 10a | Ex. 11a | Ex. 12a | Ex. 13a | Ex. 14  |
| Yellowness index.....                                             | .124      | .067    | .066    | .074    | .048    | .081    | .053    |
| Tear strength (warp/fill) grams.....                              | 320/128   | 640/416 | 576/368 | 416/288 | 512/352 | 352/272 | 512/352 |
| Tensile strength (fill) pounds.....                               | 75        | 22      | 24      |         |         |         |         |
| Dry wrinkle recovery (warp-fill) degrees.....                     | 296       | 293     | 292     | 307     | 309     | 293     | 293     |
| Durable press rating tumble dry/spin dry.....                     | 3.7/3.3   | 3.4/3.2 | 3.4/3.1 |         |         |         |         |
| Damage caused by retained chlorine, percent loss in strength..... | 4.95      | Nil     | Nil     |         |         |         |         |

A convenient method for introducing the boron salts is to add them directly to the treating bath. However, no loss in efficiency was noted when the salt was added either to the durable press finish or to the glyoxal or to the other of the raw materials used to make the durable press finish, i.e., urea or formaldehyde.

**Effect of Boric Acid Salts on Fabric Discoloration and Fabric Strength**

series, Examples 15a-17a, showed the effect of sodium tetraborate and boric acid on fabric properties and the second series, Examples 25a and 26a, showed the effect of sodium tetraborate on fabric properties using another commercial durable press finish, American Cyanamid Company's "Aerotex" 101.

Fabric performance properties are summarized in Table V below.

TABLE IV.—TREATING BATH FORMULATION

| Ingredients                                                              | Composition, percent by weight |        |        |        |        |        |        |        |        |        |        |        |
|--------------------------------------------------------------------------|--------------------------------|--------|--------|--------|--------|--------|--------|--------|--------|--------|--------|--------|
|                                                                          | Ex. 15                         | Ex. 16 | Ex. 17 | Ex. 18 | Ex. 19 | Ex. 20 | Ex. 21 | Ex. 22 | Ex. 23 | Ex. 24 | Ex. 25 | Ex. 26 |
| Durable press finish (Permafresh 183, Sun Chemical Company).....         | 17.8                           | 17.8   | 17.8   | 17.8   | 17.8   | 17.8   | 17.8   | 17.8   | 17.8   | 17.8   | 17.8   | 17.8   |
| Modified zinc nitrate catalyst (Catalyst X-4, Sun Chemical Company)..... | 3.2                            | 3.2    | 3.2    | 3.2    | 3.2    | 3.2    | 3.2    | 3.2    | 3.2    | 3.2    | 3.2    | 3.2    |
| Polyethylene softener (Mykon SF, Sun Chemical Company).....              | 1.8                            | 1.8    | 1.8    | 1.8    | 1.8    | 1.8    | 1.8    | 1.8    | 1.8    | 1.8    | 1.8    | 1.8    |
| Nonionic surfactant (Tergitol 15-S-9, Union Carbide Corp.).....          | 0.1                            | 0.1    | 0.1    | 0.1    | 0.1    | 0.1    | 0.1    | 0.1    | 0.1    | 0.1    | 0.1    | 0.1    |
| Sodium tetraborate.....                                                  |                                |        |        |        |        | 0.5    |        |        |        |        |        | 0.5    |
| Sodium metaborate.....                                                   |                                |        |        |        |        |        | 0.5    |        |        |        |        |        |
| Sodium perborate.....                                                    |                                |        |        |        |        |        |        | 0.5    |        |        |        |        |
| Potassium tetraborate.....                                               |                                |        |        |        |        |        |        |        | 0.5    |        |        |        |
| Potassium pentaborate.....                                               |                                |        |        |        |        |        |        |        |        | 0.5    |        |        |
| Ammonium borate.....                                                     |                                |        |        |        |        |        |        |        |        | 0.5    |        |        |
| Ammonium pentaborate.....                                                |                                |        |        |        |        |        |        |        |        |        | 0.5    |        |
| Boric acid.....                                                          |                                |        |        |        |        | 0.5    |        |        |        |        |        |        |
| Distilled water.....                                                     | 77.1                           | 76.6   |        |        |        |        |        |        |        | 77.1   | 76.6   |        |
| Durable press finish (Aerotex 101, American Cyanamid Company).....       |                                |        |        |        |        |        |        |        |        | 17.8   | 17.8   |        |

TABLE V.—FABRIC PERFORMANCE PROPERTIES

| Property                             | Examples |         |         |         |         |         |         |         |         |         |         |         |
|--------------------------------------|----------|---------|---------|---------|---------|---------|---------|---------|---------|---------|---------|---------|
|                                      | 15a      | 16a     | 17a     | 18a     | 19a     | 20a     | 21a     | 22a     | 23a     | 24a     | 25a     | 26a     |
| Yellowness index.....                | .134     | .080    | .084    | .083    | .069    | .069    | .076    | .078    | .148    | .135    | .041    | .032    |
| Tear strength warp/fill (grams)..... | 384/256  | 496/336 | 432/272 | 416/288 | 512/336 | 496/320 | 480/352 | 448/320 | 384/288 | 368/240 | 608/415 | 656/464 |
| Dry wrinkle recovery (degrees).....  | 297      | 285     | 289     | 288     | 277     | 284     | 280     | 285     | 283     | 280     | 280     | 258     |

NOTE.—The curing temperature for Examples 25a and 26a was 320° F.

In accord with the invention, the presence of certain boric acid salts in treating baths, containing commercial glyoxal-based durable press finishes, beneficially reduces fabric discoloration that is normally associated with this type of fabric treatment. They also significantly improve the fabric strength properties.

White cotton 136 × 64 broadcloth desized, scoured, bleached and mercerized was padded with the treating baths detailed in Table IV, and identified as Examples 15-26, using a laboratory padder at a wet pick-up of 75 percent. The fabrics were then placed on pin tenter frames, dried at 300°F. for 1.5 minutes and cured at 340°F. for 15 minutes, except for the fabrics of Examples 25a and 26a which were cured at 320°F. for 15 minutes in a laboratory oven.

Three series of experiments were performed to illustrate the degree of improvement rendered. The first

With the exception of the treatments containing the ammonium borates, the difference in each series between the control treatment and the treatments containing boron salts show the significant decrease in fabric discoloration and the increase in fabric strength that are effected by the presence of boron-containing materials. On the basis of over-all performance, sodium tetraborate and sodium metaborate are to be preferred.

Although there is a slight decrease in durable press properties (dry wrinkle recovery), this deficiency can be overcome by altering the composition of the treating bath as will be seen subsequently.

**Effect of Concentration of Sodium Tetraborate and Sodium Metaborate on Fabric Discoloration and Fabric Strength**

The degree of improvement in fabric discoloration and fabric strength is effected by the concentration of

sodium tetraborate or sodium metaborate in the treating bath. Following are examples which show the degree by which discoloration and strength are effected.

White cotton broadcloth desized, scoured, bleached and mercerized was padded (Examples 27 through 36; summarized in Table VI) through a laboratory padder at a wet pick-up of 75 percent. The fabrics were then placed on pin tenter frames, dried at 300°F. for 1.5 minutes and cured to 1.5 and 15.0 minutes at 340°F. in a laboratory oven. "Permafresh" 183 was the commercial glyoxal-based durable press finish used in these experiments.

The first series, Examples 27a-31a, showed the effect of the concentration of sodium tetraborate. The second series, Examples 32a-36a, showed the effects of sodium metaborate concentration. Fabric performance properties are summarized in Tables VII and VIII below.

coloration is obtained.

Effect of Catalyst Concentration On The Fabric Performance Properties of Fabric Treated With A Glyoxal-Based Durable Press Finish In The Presence of Sodium Tetraborate

White cotton broadcloth desized, scoured, bleached and mercerized was padded (Examples 37 through 40; summarized in Table IX) through a laboratory padder at a wet pick-up of 75 percent. The fabrics were then placed on pin tenter frames, dried at 300°F. for 1.5 minutes and cured for 1.5 and 15.0 minutes at 340°F. in a laboratory oven. "Permafresh 183" was the commercial glyoxal-based curable press finish used in these experiments.

Examples 37a-40a, showed the effect of catalyst concentration in the presence of sodium tetraborate. Fabric performance properties are summarized in Tables X and XI below.

TABLE VI.—TREATING BATH FORMULATION

| Ingredients                                                         | Compositions, percent by weight |        |        |        |        |        |        |        |        |        |
|---------------------------------------------------------------------|---------------------------------|--------|--------|--------|--------|--------|--------|--------|--------|--------|
|                                                                     | Ex. 27                          | Ex. 28 | Ex. 29 | Ex. 30 | Ex. 31 | Ex. 32 | Ex. 33 | Ex. 34 | Ex. 35 | Ex. 36 |
| Durable press finish (Permafresh 183, Sun Chemical Company)         | 17.8                            | 17.8   | 17.8   | 17.8   | 17.8   | 17.8   | 17.8   | 17.8   | 17.8   | 17.8   |
| Modified zinc nitrate catalyst (Catalyst X-4, Sun Chemical Company) | 3.2                             | 3.2    | 3.2    | 3.2    | 3.2    | 3.2    | 3.2    | 3.2    | 3.2    | 3.2    |
| Polyethylene softener (Mykon SF, Sun Chemical Company)              | 1.8                             | 1.8    | 1.8    | 1.8    | 1.8    | 1.8    | 1.8    | 1.8    | 1.8    | 1.8    |
| Nonionic surfactant (Tergitol 16-S-9, Union Carbide Corp.)          | 0.1                             | 0.1    | 0.1    | 0.1    | 0.1    | 0.1    | 0.1    | 0.1    | 0.1    | 0.1    |
| Sodium tetraborate                                                  |                                 |        |        | 0.25   | 0.50   | 0.75   | 1.00   |        | 0.25   | 0.50   |
| Sodium metaborate                                                   |                                 |        |        |        |        |        |        | 0.25   | 0.50   | 0.75   |
| Distilled water                                                     | 77.1                            | 76.85  | 76.6   | 76.35  | 76.1   | 77.1   | 76.85  | 76.6   | 76.35  | 76.1   |

TABLE VII.—FABRIC PERFORMANCE PROPERTIES AT A CURE TIME OF 1.5 MINUTES AT 300° F.

| Property                                                      | Treatment |         |         |         |         |         |         |         |         |         |
|---------------------------------------------------------------|-----------|---------|---------|---------|---------|---------|---------|---------|---------|---------|
|                                                               | Ex. 27a   | Ex. 28a | Ex. 29a | Ex. 30a | Ex. 31a | Ex. 32a | Ex. 33a | Ex. 34a | Ex. 35a | Ex. 36a |
| Yellowness index                                              | .040      | .036    | .041    | .035    | .044    | .043    | .049    | .036    | .039    | .040    |
| Tear strength (warp/fill) grams                               | 560/368   | 576/416 | 688/480 | 816/544 | 864/624 | 560/345 | 650/460 | 740/500 | 805/570 | 895/705 |
| Tensile strength (fill) pounds                                | 20        | 25      | 25      | 27      | 32      | 19      | 22      | 25      | 28      | 31      |
| Dry wrinkle recovery (warp-fill) degrees                      | 293       | 286     | 274     | 269     | 239     | 295     | 282     | 283     | 280     | 244     |
| Durable press rating (tumble dry/spin dry)                    | 3.6/3.3   | 3.4/3.1 | 3.2/2.8 | 3.1/2.3 | 2.7/2.2 | 3.6/3.2 | 3.4/3.1 | 3.4/3.1 | 3.1/2.9 | 3.1/2.5 |
| Damage caused by retained chlorine (percent loss in strength) | Nil       | Nil     | 6.7     | 4.1     | Nil     | Nil     | 4.5     | 2.8     | 6.5     | 9.0     |

TABLE VIII.—FABRIC PERFORMANCE PROPERTIES AT A CURE TIME OF 15 MINUTES AT 340° F.

| Property                                                     | Treatment |         |         |         |         |         |         |         |         |         |
|--------------------------------------------------------------|-----------|---------|---------|---------|---------|---------|---------|---------|---------|---------|
|                                                              | Ex. 27a   | Ex. 28a | Ex. 29a | Ex. 30a | Ex. 31a | Ex. 32a | Ex. 33a | Ex. 34a | Ex. 35a | Ex. 36a |
| Yellowness index                                             | .135      | .099    | .076    | .092    | .099    | .012    | .075    | .071    | .077    | .084    |
| Tear strength (warp/fill) grams                              | 432/272   | 448/304 | 544/336 | 656/400 | 672/432 | 580/315 | 505/256 | 630/363 | 630/425 | 752/452 |
| Tensile strength (fill) pounds                               | 16        | 18      | 20      | 22      | 25      | 19      | 17      | 21      | 22      | 25      |
| Dry wrinkle recovery (warp-fill) degrees                     | 284       | 292     | 280     | 273     | 266     | 296     | 291     | 285     | 289     | 274     |
| Durable press rating, tumble dry/spin dry                    | 3.6/3.3   | 3.5/3.2 | 3.5/3.2 | 3.4/3.1 | 3.4/3.0 | 3.5/3.2 | 3.4/3.2 | 3.4/3.2 | 3.4/3.1 | 3.1/3.0 |
| Damage caused by retained chlorine, percent loss in strength | Nil       | 2.9     | 5.0     | 2.5     | Nil     | Nil     | 4.8     | 9.8     | Nil     | Nil     |

Although the higher the concentration of the sodium borates in the treating bath the higher the strength properties of the fabric, the optimum concentration in relation to fabric discoloration is 0.5 weight percent. At this concentration, the minimum amount of fabric dis-

TABLE IX  
TREATING BATH FORMULATION

| EXAMPLES        | 37   | 38   | 39   | 40   |
|-----------------|------|------|------|------|
| Distilled Water | 77.8 | 76.8 | 75.8 | 73.8 |
| Permafresh 183  | 17.8 | 17.8 | 17.8 | 17.8 |

|                                               |     |     |     |     |
|-----------------------------------------------|-----|-----|-----|-----|
| Tergitol 15-S-9                               | 0.1 | 0.1 | 0.1 | 0.1 |
| Mykon SF                                      | 1.8 | 1.8 | 1.8 | 1.8 |
| Sodium Tetaborate                             | 0.5 | 0.5 | 0.5 | 0.5 |
| Modified Zinc Nitrate Catalyst (catalyst X-4) | 2.0 | 3.0 | 4.0 | 6.0 |

said solution also containing formaldehyde and in the proportions of 1 mole of glyoxal to 2 moles of formaldehyde, adjusting the pH of said solution to pH 5.5, prior to forming said reaction product, and then adding

TABLE X.—FABRIC PERFORMANCE PROPERTIES AT A CURE TIME OF 1.5 MINUTES AT 340° F.

| Property                                                     | Treatment |         |         |         |
|--------------------------------------------------------------|-----------|---------|---------|---------|
|                                                              | Ex. 37a   | Ex. 38a | Ex. 39a | Ex. 40a |
| Yellowness index                                             | .026      | .022    | .030    | .038    |
| Tear strength (warp/fill) grams                              | 944/768   | 800/656 | 704/512 | 608/448 |
| Tensile strength (fill) pounds                               | 37        | 32      | 25      | 23      |
| Dry wrinkle recovery (warp-fill) degrees                     | 248       | 260     | 280     | 295     |
| Durable press rating tumble dry/spin dry                     | 2.5/2.4   | 3.0/2.8 | 3.4/2.9 | 3.4/3.2 |
| Damage caused by retained chlorine, percent loss in strength | 3.5       | Nil     | 12.5    | Nil     |

TABLE XI.—FABRIC PERFORMANCE PROPERTIES AT A CURE TIME OF 15 MINUTES AT 340° F.

| Property                                                     | Treatment |         |         |         |
|--------------------------------------------------------------|-----------|---------|---------|---------|
|                                                              | Ex. 37a   | Ex. 38a | Ex. 39a | Ex. 40a |
| Yellowness index                                             | .067      | .053    | .059    | .130    |
| Tear strength (warp/fill) grams                              | 672/432   | 608/464 | 544/384 | 480/336 |
| Tensile strength (fill) pounds                               | 27        | 26      | 23      | 19      |
| Dry wrinkle recovery (warp-fill) degrees                     | 280       | 280     | 290     | 294     |
| Durable press rating tumble dry/spin dry                     | 3.2/2.9   | 3.3/2.9 | 3.4/3.0 | 3.3/3.2 |
| Damage caused by retained chlorine, percent loss in strength | Nil       | 3.7     | 1.0     | Nil     |

The use of the boron salts slightly effects the effectiveness of the catalyst. The slight loss in catalyst efficiency can be overcome by increasing the catalyst concentration by approximately 1 percent. The data indicated that 4 percent by weight of the catalyst is optionally employed. This will, of course, differ with different treating bath compositions and different glyoxal-based durable press finishes.

What is claimed is:

1. In the process for crease-proofing cellulose-containing textile fabric wherein the reaction product of glyoxal, urea and formaldehyde is applied to said fabric in an acidic medium and thereafter cured to impart crease-resistance to said fabric, the improvement in making said reaction product comprising adding sodium metaborate to an aqueous solution of glyoxal,

proportionately 1 mole of urea to said solution and changing the pH of the solution of pH 7 which is maintained during the formation of said reaction product, said sodium metaborate being added to said glyoxal in an amount ranging between about 0.5 and 20 weight percent based on the weight of the total solution.

2. The process of claim 1 wherein said sodium metaborate is added in an amount ranging between about 6 and 14 weight percent.

3. A process according to claim 1 wherein said textile fabric is a blend of polyester and cotton.

4. A process according to claim 1 wherein said textile fabric is cotton.

5. A process according to claim 1 wherein said textile fabric is rayon.

\* \* \* \* \*